

April 20, 1937.

A. L. HELWITH

2,077,692

FABRIC

Filed May 3, 1934

*Fig. 1*



*Fig. 2*



*Fig. 3*



*Alfred L. Helwith*  
INVENTOR:  
BY  
*Miss Schumacher*  
ATTORNEY

## UNITED STATES PATENT OFFICE

2,077,692

## FABRIC

Alfred L. Helwith, Larchmont, N. Y.

Application May 3, 1934, Serial No. 723,656

6 Claims. (Cl. 139—420)

This invention relates to textile fabrics and methods of making the same. While the invention may be of general application to textile fabrics, it is particularly of advantage in a rayon 5 fabric.

One object of the invention is to provide a novel ribbed textile fabric and method of making the same, with special reference to a rayon fabric.

10 It is well known that rayon fabrics are most desirable when wholly and uniformly lusterless, and this invention is intended to provide a fabric of this character. Since rayon yarns are relatively translucent, the production of a suitable 15 ribbed rayon fabric has not been known heretofore.

It is an accepted fact that the composition 20 yarns, such as those of which rayon is made, are produced free of twist, and that to provide a twist in such yarns increases the cost of the 25 fabric to an extent dependent upon the degree of twist provided in the yarn. With this factor in mind, this invention aims to provide an improved ribbed inexpensive fabric.

25 Then again, while fabrics having pronounced ribs resulting in rough or irregular surfaces for the fabric are well known, it is nevertheless accepted that a fabric having a substantially smooth surface affords the maximum wear, and 30 is relatively easiest to keep clean in course of normal use.

It is therefore an object of the invention to 35 provide an improved ribbed, uniformly dull fabric, the ribs being so slight as to permit the fabric to have a substantially continuously smooth 40 surface throughout; and, further that said fabric shall be inexpensive, and adapted to be made by standard machinery and in a very simple and cheap manner.

40 Other objects and advantages of the invention will become apparent as the specification proceeds.

With the aforesaid objects in view, the invention 45 consists in the novel combinations and arrangements of parts hereinafter described in their preferred embodiments, pointed out in the subjoined claims, and illustrated in the annexed drawing, wherein like parts are designated by 50 the same reference characters throughout the several views.

In the drawing:

Figure 1 is a considerably magnified plan view 55 of a section of a textile fabric, embodying the invention.

Fig. 2 is a similar view of a modification of the invention.

Fig. 3 is a plan view of a section of a textile fabric, embodying the invention and showing the normal appearance thereof.

The advantages of the invention as here outlined are best realized when all of its features and instrumentalities are combined in one and the same structure, but, useful devices may be produced embodying less than the whole.

It will be obvious to those skilled in the art to which the invention appertains, that the same may be incorporated in several different constructions. The accompanying drawing, therefore, is submitted merely as showing the preferred 10 exemplification of the invention.

Referring in detail to the drawing, 10 denotes a section of a textile fabric embodying the invention. The same may be constructed of a suitable, preferably regular weave, and is desirably 20 of uniform color throughout. Further, the fabric 10 is characterized by a ribbed appearance as shown at 11, whereby the attractiveness and hence the value of the fabric are enhanced. The ribbed effect may be made to extend either across 25 the warp or across the weft, as may be desired, but the former is preferable.

According to the invention, the fabric 10, as shown in Fig. 1, may have a weft including uniformly spaced weft yarns 12 which are desirably 30 of the same weight and color throughout. The warp may include uniformly spaced alternately consecutive warp yarns 13 and 14 which are desirably of one color. It will be seen, however,

35 that the yarns 13 and 14 are of different weight, and are more closely spaced than the filling yarns. Thus the ribs 11 are caused to extend transversely of the warp as shown in Fig. 3. In

the case of a rayon fabric, all of the yarns 12, 13 40 and 14 may be lusterless, and if the difference in weight of the yarns 13, 14 is substantial, a distinct mechanical ribbed effect is produced, which is rendered extremely close and highly attractive

45 by reason of the fact that the yarns 13, 14 follow each other in single succession. It will be noted that the yarns 14 may have a weight double or triple that of the yarn 13, while the latter may desirably be of the same or approximately

50 the same weight as the weft yarns 12. As all the yarns 12, 13 and 14 consist preferably of the same material, a very neat fabric 10 is obtained, in which the ribs are in such close proximity to each other as to afford a practically smooth surface fabric 10. Since the ribs 11 are each provided by a single yarn 14, uniformity is assured

5

10

15

20

25

30

35

40

45

50

55

in appearance in softness and in the relative smoothness and thickness of the fabric.

It may be noted that by this invention, individual or single ply yarns can be used throughout, instead of the more expensive multi ply yarns. The latter necessarily require a relatively high twist to produce a workable thread, and it is an object herein to reduce the amount of twist required in the yarns of my fabric. As the heavier yarns are less translucent than the lighter yarns, the ribbed effect is further accentuated.

I have found, however, that it is preferable and less expensive to construct the fabric 10 with a lesser difference in weight between the yarns 13 and 14, for two reasons. In the first place, the comparative smoothness of the fabric surface may be further increased, and in the second place, changes in length due to shrinkage and the like as between yarns 13 and 14 are reduced. Thus the fabric 10 may be maintained relatively smooth without requiring special treatment of the yarns 13 and 14 to produce an even shrinkage. This I accomplish by utilizing warp 25 yarns such that the yarn 14 is less than twice the weight of the yarns 13, and preferably not more than twenty to sixty percent heavier than the latter, it being understood that if the relatively 30 smallest available difference in the weight of the yarns is utilized, the tension on the yarns may be equal for weaving the fabric on a single beam. However, this result tends to cause the ribbed appearance to disappear. A second cause which 35 tends toward disappearance of the ribbed effect is especially due to composition or rayon yarns, which are largely translucent.

To overcome these drawbacks, I utilize yarns 14 which have twist, and thus optically supplement the effect of the relatively small difference 40 in weight between the yarns 13, 14, to render the ribbed appearance sufficiently distinctive. If a high or tight twist were required, the rayon fabric would become so expensive as to counterbalance its advantages, and would acquire undesirable crinkly effects. However, I have found 45 that a comparatively slight twist of say ten to twenty-five turns per inch is sufficient and may be termed moderate, and since the yarns 14 are only a little more than one-fourth or one-third 50 the weight of the fabric 10, the increase in cost of the fabric is relatively small. The foregoing principles are also applicable to other textiles, such as cotton fabrics, but as noted, the advantages are most clear in a composition of rayon 55 fabric.

The size of the yarns is more important when referring to the twisted yarns 14, because twisting tends to increase the size of these yarns. Nevertheless the translucency of the yarns 14 is 60 reduced by twisting, and both the size and translucency of the yarn 14, in conjunction with the twist thereof, are important factors in producing the ribbed effect in the fabric 10. By the term textile fabric is meant a fabric such as a 65 taffeta, or the like, adapted to be made into garments.

In Fig. 2 is shown a modification of the invention, including a fabric 15 substantially similar to the fabric 10 in appearance, and differing therefrom in construction solely in that the warp yarns 16 corresponding to yarns 13 are twisted, while the yarns 17 corresponding to the 70 yarns 14 are not twisted, but straight or plain. The ratio of weights may be the same as hereinbefore described, and the yarns 16 may have the

same but preferably a considerably greater twist than the yarns 14. While the fabric 15 will not afford as distinct a rib as the fabric 10, it is nevertheless shown as a possible construction within the scope of the invention.

It will be understood that while the fabric provided by my invention preferably consists of uni-colored or shaded yarns, it is not limited thereto, as alternately consecutive warp yarns may additionally be of different shade. An important element of the fabric lies, however, in the fact that it is of one color. Likewise certain yarns may be of a different material than other yarns. The twist of the alternate warp yarns may be in the same or in opposite directions as desired; and further, the invention includes the principle of a textile fabric having warp yarns of the same or substantially the same weight where the singly successive yarns are arranged plain and twisted as shown in Fig. 1. However, where warp yarns of different weights are used, it is contemplated that the ratio of weights shall in general be such as to produce a relatively smooth surface fabric. If the plain yarns such as 13 are produced by such a process, as naturally to possess a very slight 25 twist, say between two and a half to five times per inch, the yarns 13 and 14 may be laid so that the twist is in opposite directions; but such yarns can be regarded as plain for most practical purposes. Although reference has been made herein 30 to warp yarns such as 13 and 14 arranged in consecutive alternation, the principle of the fabric 10 can be employed to produce certain desirable though much less pronounced attractive effects as where the yarns 13, 14 are laid in an alternate 35 two and two arrangement, and with the same weave as shown. Finally, it will be noted that different features herein pointed out may be combined and arranged in various other ways to produce other fabrics.

It will be appreciated that various changes and modifications may be made in the device as shown in the drawing, and that the same is submitted in an illustrative and not in a limiting sense, the scope of the invention being defined in the following claims.

I claim:

1. A taffeta-like rayon fabric having a warp and weft interwoven in a regular order and arrangement throughout the fabric, said yarns being lusterless and all of one color, the warp consisting of relatively light and heavy yarns arranged in consecutive alternation, one of the series of light and heavy yarns consisting of twisted yarns, the weft consisting of relatively 55 light yarns, and there being more warp than weft yarns per inch, as set forth.

2. A textile fabric for garments, having a regularly interwoven warp and weft and the warp yarns being more closely spaced than the weft 60 yarns, said warp consisting of a series of relatively light and heavy yarn elements, the light and heavy elements being arranged in alternation, and one of said series of light and heavy elements having a twist, as set forth.

3. A rayon textile fabric having a regularly interwoven warp and weft, the warp yarns being more closely spaced than the weft yarns, all of the warp and weft yarns being of one dull color, the warp consisting of light and heavy yarns in 70 single consecutive alternation, the heavy yarns being moderately twisted and the light yarns being relatively plain, as set forth.

4. A rayon textile fabric having an interwoven warp and weft, the warp yarns being more closely 75

- spaced than the weft yarns, all of said yarns being dull and of one color, the warp yarns including 5  
yarns of different weights such that the heavy  
yarns are from 20 to 100 percent greater in weight  
than the lighter yarns of the warp, the said  
lighter yarns and the weft yarns being of approxi-  
mately the same weight, the light and heavy  
warp yarns being arranged in single consecutive  
alternation, the heavy warp yarns having a twist  
10 of between 10 and 20 turns per lineal inch, as set  
forth.
5. A rayon textile fabric having a warp and a  
weft, the warp yarns being more closely spaced  
than the filling yarns, the warp including plain  
15 and moderately twisted yarns arranged in single

succession, the twisted yarns being at least  
twenty percent heavier than the plain warp yarns  
to such a degree that the fabric has nevertheless  
a substantially smooth surface.

6. A rayon textile fabric of the character de-  
scribed including an interwoven warp and weft,  
the yarns of the warp being more closely spaced  
than those of the weft, the warp yarns including  
yarns of different weights such that the heavy  
yarns are approximately twenty percent greater 10  
in weight than the lighter yarns of the warp, the  
light and heavy yarns being disposed in alterna-  
tion, and one of the series of light and heavy yarns  
having a relatively moderate twist.

ALFRED L. HELWITH. 15